

Patented Mar. 4, 1924.

1,485,790

# UNITED STATES PATENT OFFICE.

KARL LÜTTIN, OF BASEL, SWITZERLAND, ASSIGNOR TO J. R. GEIGY A. G., OF BASEL SWITZERLAND, A CORPORATION OF SWITZERLAND.

## DYE SOLUTION AND PROCESS FOR MAKING AND UTILIZING SAME.

No Drawing.

Application filed June 26, 1922. Serial No. 571,098.

To all whom it may concern:

Be it known that I, KARL LÜTTIN, a citizen of the Swiss Republic, and resident of Basel, Switzerland, have invented Dye Solutions and Processes for Making and Utilizing Same, of which the following is a full, clear, and exact specification.

As well known, the organic dyestuffs of basic or acid nature are utilized for dyeing textile fibres, by dyeing in a neutral or slightly acid solution, with or without mordant, at a relatively high temperature, or by fixing the printed dyes by steaming.

I have found that dyeings can be obtained at ordinary temperatures, which are fast to washing and rubbing, if dye solutions are employed which contain, with or without a thickening substance, about 10 to 20% of at least one chloracetic acid, as monochloracetic acid, dichloracetic acid, trichloracetic acid, or a mixture of several of these acids. When used in printing, these solutions show the advantage that the steaming can be omitted. The present invention relates consequently to dye solutions characterized by a content of one or several of the specified acids, to a process for the manufacture of these dye solutions, to a process for producing with these dye solutions dyeings and printings on textile fibres and other substances, as wood, paper, feathers, leather, furs, straw, tagal, artificial substances etc. and finally to the dyeings and printings obtained with these dye solutions.

The process for the manufacture of the said dye solutions can be guided by the dyeing quality of the dyestuff, in as far as basic dyestuffs require an addition of tannin for their employ on cotton.

The essential condition for the manufacture of these solutions is that the dyestuffs have been made and remain entirely soluble.

The following examples illustrate the preparation and the composition of the new dye solution and their use for dyeing and printing purposes.

### Example I.

1 gr. of a basic dyestuff is dissolved in 5 gr. acetic acid of 40 per cent and 20 gr. of boiling water; to the solution thus obtained there are added 52 g. of tragacanth gum thickening and 2 gr. of tannin, 20 gr. of monochloracetic acid are then added

and after dissolution the dye-solution is ready for use.

If instead of monochloracetic acid, there is employed lactic acid, this latter is used in form of a solution of a specific gravity of 1.21.

After printing the fabric with this dye, the fabric is dried and passed, without steaming, through a cold or hot bath of tartar emetic containing, as usual, 10 gr. of tartar emetic to a liter of water. Afterwards the fabric is well rinsed and soaped. The dyestuff is regularly and quickly fixed and cannot be removed by rubbing.

### Example II.

For the merchandises half of silk and half of cotton there is prepared in the same manner as for the cotton a dyeing bath having the following composition:

|                                             |    |
|---------------------------------------------|----|
| 1 gr. of basic dyestuff is dissolved in     | 75 |
| 5 gr. of acetic acid of 40 per cent and     |    |
| 20 gr. of boiling water and there are added |    |
| 42 gr. of cold water                        |    |
| 10 gr. of tragacanth gum thickening         | 80 |
| 2 gr. of tannin and                         |    |
| 20 gr. of monochloracetic acid.             |    |

The fabric pieces are impregnated with this dyeing bath in a fulling mill and pressed out in such a manner that in the moistened state they show an increase of weight of 100 per cent. After they have been well dried, they are passed, without steaming, through the usual bath of tartar emetic, rinsed and soaped.

### Example III.

For wool and silk the dye solution is prepared, in a manner similar to that of Example I and formed of

|                                         |    |
|-----------------------------------------|----|
| 1 gr. of acid dyestuff dissolved in     | 85 |
| 5 gr. of acetic acid of 40 per cent and |    |
| 20 gr. of hot water and there are added |    |
| 44 gr. of cold water                    |    |
| 10 gr. of tragacanth gum thickening and | 90 |
| 20 gr. of monochloracetic acid.         |    |

The fabric is dyed in pieces in a fulling mill and the dyeing terminated without steaming.

The new dye solutions are utilizable not only in the industry for dyeing and printing textile fabrics, but can also owing to their stability and their property of being easily

manageable be used for purposes of industrial art, as they permit a hitherto unknown fast dyeing of textile fabrics by applying the dye solution by painting or sprinkling. 5 They are utilizable in the same manner for paper, straw, leather, wood, feathers, furs, artificial substances etc.

What I claim is:

1. As a new article of manufacture, a 10 new dye solution containing at least one chloracetic acid.
2. As a new article of manufacture, a new dye solution containing a thickening and at least one chloracetic acid.
- 15 3. As a new article of manufacture, a new dye solution containing tannin and at least one chloracetic acid.
4. As a new article of manufacture, a new dye solution containing a thickening and tannin and at least one chloracetic acid.
- 20 5. The herein described process for the manufacture of dye solutions consisting in introducing at least one chloracetic acid into a dyestuff solution.
- 25 6. The herein described process for the manufacture of dye solutions consisting in introducing at least one chloracetic acid into a dyestuff solution containing a thickening.
- 30 7. The herein described process for the manufacture of dye solutions consisting in introducing at least one chloracetic acid into a dyestuff solution containing tannin.
8. The herein described process for the 35 manufacture of dye solutions consisting in introducing at least one chloracetic acid, into a dyestuff solution containing a thickening and tannin.
9. The herein described process for producing dyeings and printings on textile fab-

rics, paper, straw, leather, wood, feathers, furs, artificial substances etc. consisting in applying on the said merchandises, at ordinary temperature, a dye solution containing at least one chloracetic acid.

45

10. The herein described process for producing dyeings and printings on textile fabrics, paper, straw, leather, wood, feathers, furs, artificial substances etc. consisting in applying on the said merchandises at 50 ordinary temperature, a dye solution containing a thickening and at least one chloracetic acid.

50

11. The herein described process for producing dyeings and printings on textile fabrics, paper, straw, leather, wood, feathers, furs, artificial substances etc. consisting in applying on the said merchandises at ordinary temperature, a dye solution containing tannin and at least one chloracetic acid and 60 passing the merchandises subsequently, without steaming, through a bath of tartar emetic.

55

12. The herein described process for producing dyeings and printings on textile fabrics, paper, straw, leather, wood, feathers, furs, artificial substances etc. consisting in applying on the said merchandises, at ordinary temperature, a dye solution containing a thickening and tannin and at least 70 one chloracetic acid and passing the merchandises subsequently, without steaming, through a bath of tartar emetic.

65

In witness whereof I have hereunto signed my name this 13th day of June 1922, in the 75 presence of two subscribing witnesses.

KARL LÜTTIN.

Witnesses:

JULIA A. DÜRST,  
AMAND RITLER.